

## UNITED STATES PATENT OFFICE

2,173,297

## METHOD OF PERMANENT WAVING

Myles Wade Fletcher, Atlanta, Ga., assignor to  
Utility Sales Corporation, Atlanta, Ga., a corporation of Georgia

No Drawing. Application August 27, 1936,  
Serial No. 98,200

2 Claims. (Cl. 132—36)

This invention relates to a composition of chemicals that when moistened will generate sufficient heat to impart upon a prepared tress, a so-called permanent wave. A heating time of from 5 three to five minutes at a temperature of between 98° and 120° centigrade maximum is necessary to impart the proper wave to the prepared tress and this invention is a means of obtaining this condition through the use of a chemically heating 10 compound.

I have found that a mixture of copper oxide (either cupric or cuprous), potassium chlorate or perchlorate aluminum metal and ammonium chloride when moistened will generate sufficient 15 heat to impart the proper wave to a prepared tress. These chemicals may be compounded in various proportions and obtain relatively the same degree heat for the same length of time, but can also be compounded to obtain different degrees 20 of heat for different lengths of time. This latter feature is of much importance in the hair waving art, as different textures and conditions of hair require different degrees of heat and different heating times in order to obtain the best results 25 in imparting the so-called permanent wave to the hair. This heating mixture gives off no harmful gases or has no apparent damaging effect of any kind upon the tress.

Aluminum grindings, turnings, borings, etc., 30 may be obtained at a very low cost as scrap metal. Iron filings may be used as a substitute for part of the aluminum, but I find the heat more difficult to intensify and other disadvantages such as discoloration from the resulting oxidation. In the 35 use of iron a catalytic agent for oxidation, such as titanium oxide, nickel oxide, or cobalt oxide, must be employed in the mixture in order to get a sufficiently high degree of heat. Compounds may be substituted for the chlorate or perchlorate 40 having available oxygen, such as sodium peroxide or sodium perborate.

A typical mixture for waving normal medium texture hair consists of three parts potassium chlorate, one part copper oxide, one part aluminum grindings (30 mesh and finer) and one-tenth part ammonium chloride. With this mixture maximum heat of approximately 110° centigrade is obtained and when moistened by a strip of cotton flannel in contact will remain above 90° 45 centigrade for 8 minutes.

Various designs of receptacles are possible to hold this mixture and allow it to be moistened,

such as a flat bag of flannel or an envelope with impervious back and absorbent front. The ammonium chloride may be added to the mixture by moistening with a solution of same. It is desirable to employ this method as a guard against decomposition by atmospheric moisture. A very satisfactory method is to add the ammonium chloride to the waving lotion with which it is necessary to moisten the tress in order to obtain a so-called permanent wave. The merit of this 10 method is that the pad containing the chemical mixture can be moistened with the same lot to begin the heating reaction. A lotion consisting of approximately eight percent sodium sulphite, ten percent ammonium chloride and five one- 15 hundreds of one percent amyl acetate give very desirable results.

Ammonium chloride is the only salt I have found that will go into solution satisfactorily and also start the reaction between aluminum, potassium chlorate and copper oxide that will produce sufficient heat to impart the proper permanent wave to a prepared tress. Ammonium chloride plays the dual roll of being a necessary ingredient to the action of the lotion on the hair 25 and that of starting the chemical reaction.

Having thus described the invention, what I claim and desire to secure by Letters Patent is:

1. A method of waving hair by heat comprising applying thereto a dry composition comprising 30 alkali chlorate in a major amount and a mixture of powdered metal of the fineness of about 30 mesh and powdered metal oxide in substantially equivalent amounts and in total amount less than the oxidizing agent, said composition being capable of producing heat upon moistening with a solution of ammonium chloride, and then moistening the composition with said solution.

2. A method of waving hair by heat comprising applying thereto a dry composition comprising 40 alkali chlorate in major amount and a mixture of powdered metal and powdered metal oxide in substantially equivalent amounts and in total amount less than the oxidizing agent, said composition being capable of producing heat upon 45 moistening with a solution of ammonium chloride including 10 per cent. ammonium chloride, 8 per cent. sodium sulphite, 0.05 per cent. amyl acetate, balance water, and then moistening the composition with said solution.

MYLES WADE FLETCHER.